# EUROPEAN PATENT SPECIFICATION

(11) **EP 0 711 822 B1**
(45) Date of publication and mention of the grant of the patent: **13.09.2006**
(21) Application number: 95202994.0
(22) Date of filing: 06.11.1995
(51) Int. Cl.: C10M 133/02, C10M 141/10, C10M 141/06, C10M 133/06, C10M 133/16, C10M 129/40, C10M 135/02, C10M 137/02, C10M 137/04, C10M 137/08, C10N 30/06, C10N 30/12, C10N 40/20

(54) **Method of lubricating slideways**
Verfahren zur Schmierung von Gleitführungen
Procédé de lubrification de glissières

(30) Priority: 09.11.1994 JP 27518594
(43) Date of publication of application: 15.05.1996
(73) Proprietor: SHELL INTERNATIONALE RESEARCH MAATSCHAPPIJ B.V., 2596 HR Den Haag (NL)
(72) Inventor: Aoki, Nobuhiro, Yonago-shi, Tottori-ken (JP); Baba, Yoshiharu, Hatano-shi, Kanagawa-ken (JP)

(56) References cited:
- EP-A- 0 407 124
- DD-A- 63 835
- US-A- 4 740 323
- US-A- 4 822 507
- DATABASE WPI Section Ch, Week 9403 Derwent Publications Ltd., London, GB; Class E11, AN 94-023127 XP002023595 & JP-A-05 331 478 (TONEN CORP) , 14 December 1993
- DATABASE WPI Section Ch, Week 9114 Derwent Publications Ltd., London, GB; Class E11, AN 91-096926 XP002023596 & JP-A-03 039 399 (TONEN CORP) , 20 February 1991 & US-A-5 391 307 (AKIRA YAMAZAKI)

## Description

The present invention relates to a method of lubricating the slideway(s) of a machine tool or injection moulding machine and the use of a lubricating oil composition for lubricating the slideway(s) of a machine tool or injection moulding machine. The lubricating oil composition for use in the method of the present invention is more particularly for use in a machine tool for precise machining at a low feed speed.

Positioning of a machine tool table should be controlled accurately for precise machining.

However, in the case of a machine tool having a slideway, the friction in the slideway produces elastic strain in the feed systems, reducing the accuracy of positioning.

Generally, various kinds of friction reducing agents are incorporated in lubricating oil compositions for use in slideways. For example, 0.1 to 10% by weight of fat esters, fat sulphides, fatty acids and/or phosphoric esters are incorporated in a base lubricating oil.

US-A-4 822 507 discloses a method of lubricating a metal working machine which has (i) at least one sliding machine surface requiring lubication and (ii) a metal working section wherein metal is worked in contact with a metal working fluid, said method comprises applying a lubricating oil composition to said at least one sliding surface and using as said metal working fluid an aqueous working fluid composition comprising said lubricating oil composition diluted with water, said lubricating composition comprising; (A) 5 to 88% by weight of at least one oil selected from the group consisting of a mineral oil and a synthetic oil, (B) 2 to 50% by weight of a reaction product of a long chain dibasic acid having 14 to 28 carbon atoms and an alkanolamine, (C) 5 to 30% by weight of at least one extreme pressure additive selected from the group consisting of sulfurized fat and oil, a phosphate, a phosphite, and an amine salt of phosphate or phosphite (D) 5 to 30% by weight of an emulsifying agent selected from the group consisting of an anionic surface active agent, a cationic surface active agent, a nonionic surface active agent and a phosphorus-containing surface active agent.

However, conventional lubricating oil compositions have insufficient lubricity for lubricating slideways of a machine tool for precise machining. Incorporating a highly active friction reducing agent or increasing its amount was necessary for obtaining the desired lubricity. However, employing such friction reducing agent in a high concentration led to the problem of increasing the cost of such lubricating oil compositions. In addition, incorporation of a high concentration of active friction reducing agents such as fatty acids or phosphoric esters in the base oil have sometimes caused corrosion on slideways or oil supplying systems of a machine tool.

The present invention is aimed at providing the use of a lubricating oil composition of a low cost which is particularly suitable for use in a machine tool for precise machining and improves the accuracy of positioning of sliding systems in such a tool, and which is substantially non-corrosive.

In accordance with the present invention there is provided a method of lubricating the slideway(s) of a machine tool or injection moulding machine comprising lubricating said slideway(s) with a lubricating oil composition comprising
(a) a base oil comprising one or more lubricating oils selected from mineral, vegetable and synthetic lubricating oils;
(b) one or more friction reducing agents selected from phosphoric acid ester alkyl ammonium salts of the formulae:

   [(R¹O)ₙP(=O) (O⁻)₃₋ₙ] [R²ₘH₍₄₋ₘ₎N⁺]₃₋ₙ (1)

   [(R¹O)ₙP(=O) (O⁻)₃₋ₙ] [R²ₘR³₍₃₋ₘ₎HN⁺]₃₋ₙ (2)

   and fatty acids of the formulae: wherein n is 1 or 2; m is 1 to 3; p is 1 to 10; R¹ is a C₄₋₂₂ alkyl, alkenyl or alkynyl group, a C₆₋₂₄ alkylaryl group, an alkyl group to which 1 to 10 moles of polyoxyethylene is added, or an alkylaryl group to which 1 to 10 moles of polyoxyethylene is added; R² is a C₄₋₂₆ alkyl, alkenyl or alkynyl group, a C₆₋₂₄ alkylaryl group or an aryl group; R³ is a methyl or ethyl group; R⁵ is a C₇₋₂₃ alkyl, alkenyl or alkynyl group or a sulphurised C₇₋₂₃ alkyl, alkenyl or alkynyl group; R₆ is a C₁₀₋₁₈ alkyl, alkenyl or alkynyl group; and R⁷ is a C₈₋₁₈ alkyl, alkenyl or alkynyl group; and
(c) one or more linear alkyl amines selected from the amines represented by the formulae:

   R⁸ₘ-N-H₍₃₋ₘ₎ (6)
wherein m and R³ are as defined above; and R⁸ is a linear C₈₋₂₂ alkyl, alkenyl or alkynyl group, provided that R⁸ has more carbon atoms than R² when R² is a linear alkyl, alkenyl or alkynyl group.

The base oil (a) used in the present invention preferably has a kinematic viscosity of ISO VG 10 to 220 (at 40°C).

The mineral lubricating oil usable as the base oil (a) includes paraffinic and naphthenic mineral oils which are purified through solvent extraction and/or hydrogenation.

The vegetable lubricating oil includes rape seed oil, rice bran oil, soybean oil and others manufactured from vegetables.

The synthetic lubricating oil includes olefin oligomers, polybutenes, fatty acid esters such as esters of adipic, azelaic, phthalic, oleic or stearic acid, and polyol esters such as trimethyl propanol oleate, pentaerythritol oleate, neopentyl glycol oleate and trimethyl propanol isostearate.

These base oils can be used individually or in combination.

In the composition of the present invention, preferably R¹ is a C₄₋₂₀ alkyl group, a C₁₆₋₂₀ alkenyl group, a C₄₋₂₀ alkyl group to which 1 to 10 moles of polyoxyethylene is added, or a (C₁₋₁₀ alkyl)phenyl group to which 1 to 10 moles of polyoxyethylene is added; R² is a C₄₋₁₆ alkyl group or a phenyl group; R³ is a methyl group; R⁴ is a C₈₋₁₄ alkyl group or a C₁₆₋₂₀ alkenyl group; R⁵ is a C₈₋₂₀ alkyl group, a C₁₀₋₂₀ alkenyl group or a sulphurised C₁₆₋₁₈ alkenyl group; R⁶ is a C₁₀₋₁₈ alkyl group or a C₁₆₋₂₀ alkenyl group; R⁷ is a C₁₀₋₁₈ alkyl group; and R⁸ is a linear C₈₋₂₀ alkyl group or C₁₆₋₂₀ alkenyl group.

More preferably, the one or more friction reducing agents are selected from:
mono- or di-alkyl acid esters such as butyl acid phosphate, hexyl acid phosphate, octyl acid phosphate, 2-ethylhexyl acid phosphate, isodecyl acid phosphate, lauryl acid phosphate, stearyl acid phosphate, oleyl acid phosphate, polyoxyethylene alkyl ether acid phosphate, and polyoxyethylene isooctylphenyl ether acid phosphate; alkyl ammonium salts of such phosphoric acid esters obtained by neutralisation of these esters with butyl amine, dibutyl amine, octyl amine, trioctyl amine, 2-ethylhexyl amine, di-2-ethylhexyl amine, t-alkylamine represented by the formula R^{a}R^{b}R^{c}CNH₂ wherein R^{a}, R^{b} and R^{c} are alkyl groups and the total number of the carbon atoms of R^{a}, R^{b} and R^{c} is 3 to 25, isotridecyl amine, diisotridecyl amine, tridecyl amine, ditridecyl amine, dimethyl octyl amine or diphenyl amine;
phosphorous acid esters such as dioctyl, dilauryl and dioleyl phosphites; and
fatty acids such as capric, lauric, myristic, palmitic, stearic, oleic, erucic, linoleic and linolenic acids or oleic acid sulfide; N-acylsarcosines such as lauroyl, myristoyl, palmitoyl and oleoyl sarcosines; and alkylether carboxylic acids such as polyoxyethylene lauryl ether carboxylic acid, polyoxyethylene stearyl ether carboxylic acid and polyoxyethylene beef tallow ether carboxylic acid.

These friction reducing agents can be used individually or in combination.

More preferably, the one or more linear alkyl amines (c) are selected from:
octyl amine, dioctyl amine, trioctyl amine, laurylamine, myristyl amine, palmityl amine, stearyl amine, oleyl amine, dioleyl amine, distearyl amine, dimethyl stearyl amine, dimethyl oleyl amine, and dimethyl coconut amine.

The one or more friction reducing agents (b) can be used in an amount of 0.05 to 10.0% by weight, preferably 0.1 to 5.0% by weight, based on the amount of base oil (a). A lubricating oil composition containing less than 0.05% by weight of the friction reducing agent(s) (b) does not provide sufficient friction reducing effect, while a lubricating oil composition containing more than 10.0% by weight of the component (b) may corrode materials of a machine tool.

The amount of the one or more linear alkyl amines (c) is 0.1 to 20% by weight, preferably 1 to 10% by weight, based on the amount of the friction reducing agent (b). When the amount of the linear alkyl amine (c) is less than 0.1% by weight, the purpose of the present invention cannot be achieved. On the other hand, when more than 20% by weight of the linear alkyl amine (c) is incorporated, the linear alkyl amine (c) is not dissolved well in the base oil (a) when the base oil (a) is a mineral lubricating oil and the acid phosphoric ester, phosphorous ester or fatty acid used as the friction reducing agent (b) has a linear alkyl group. In addition, the activity of the friction reducing agent (b) is lowered and lubricity of the lubricating oil composition is adversely affected.

A publicly known lubricity improver can be optionally incorporated in the lubricating oil composition of the present invention. The following additives are mentioned as the examples of the lubricity improver:
oiliness improvers, extreme pressure additives and/or anti-wear additives; for example, higher alcohols, metal soaps of fatty acids, animal or vegetable fats and oils, fatty acid esters, sulphides of animal or vegetable fats and oils, ester sulphides, trialkyl phosphates, tricresyl phosphates, trialkyl phosphites, organomolybdenum friction reducing agents and zinc alkyl dithiophosphates.

In addition, antioxidants, rust inhibitors, detergents, viscosity index improvers, pour point depressants, metal deactivators, defoamers, demulsifiers and/or tackifiers, usually used as lubricating oil additives, can be optionally incorporated.

The lubricating oil composition of the present invention, wherein specific additives are combined with conventional ones, provides an excellent positioning accuracy which could not be obtained by lubricants containing a known additive individually. Therefore, machining accuracy of a machine tool can be remarkably improved by using the lubricating oil composition of the present invention. The lubricating oil composition can be also preferably used as a lubricating oil for slideways of an injection moulding machine which is required to mould materials precisely.

Therefore in accordance with the present invention there is provided a method of lubricating the slideway(s) of a machine tool or injection moulding machine comprising lubricating said slideway(s) with a lubricating oil composition according to the present invention.

In accordance with the present invention there is further provided use of a lubricating oil composition as defined in the present invention for lubricating the slideway(s) of a machine tool or injection moulding machine.

In addition, the concentration of additives such as friction reducing agents can be reduced, while it was previously necessary to add conventional friction reducing agent in a high concentration for obtaining a desired lubricating performance. Therefore, the lubricating oil composition of the present invention can effectively prevent parts of a machine from corrosion caused by adding friction reducing agent in a high concentration. Further, the lubricating oil composition is inexpensive compared with conventional lubricating oil compositions.

The present invention will now be described by way of example with reference to the following working

### examples:

### Examples 1 to 8 and Comparative Examples 1 to 12 Preparation of Sample Oil Compositions

A lubricating oil having a kinematic viscosity of ISO VG 68, a viscosity index of 110, a pour point of -15°C, a total acid number of 0.00 mgKOH/g and a sulphur content of 0.5% by weight was used as a base oil (a).

The following compounds were used as additives:
sulfurised lard (from Dainippon Ink and Chemicals, Ltd.),
oleic acid (from Unichema International),
alkyl ammonium salt of phosphoric acid ester obtained by mixing octyl acid phosphate (from Asahi Denka Kogyo K.K.) and ditridecyl amine (from BASF AG) (hereinafter "amine salt of phosphoric acid ester 1"),
alkyl ammonium salt of phosphoric acid ester obtained by mixing octyl acid phosphate (from Asahi Denka Kogyo K.K.) and di-2-ethylhexyl amine (from BASF AG) (herein after "amine salt of phosphoric acid ester 2"),
alkyl ammonium salt of phosphoric acid ester obtained by mixing hexyl acid phosphate (from A. & W Co.) and tertiary C₁₂₋₁₄ alkyl amine (from Rohm & Haas Company) (hereinafter "amine salt of phosphoric acid ester 3"),
   tricresyl phosphate (from Ciba-Geigy Limited), and 2-ethylhexyl amine (from BASF AG),
   dioleyl amine (from Nippon Oil and Fats Co. Ltd.), lauryl amine (from Kao Corporation),
   oleyl amine (from Hoechst AG), and
   tertiary C₁₆₋₂₂ alkyl amine (from Rohm & Haas Company).

### Positioning Test Procedure

A positioning test was carried out in accordance with the procedure of least input increment feed test of vertical type machining centre set forth in JIS B6338 Para. 2.8.

The machining centre was commanded through numeral control so as to feed 25 times by 1 µm/time at intervals of 10 seconds to the plus direction on Y axis, and then, to feed to the minus direction in the same manner. Actual displacement length was measured by a laser beam length measuring instrument. The accuracy of the response of the feed of the machine table to a series of the numeral control commands was measured for the sample oil compositions of these examples and comparatives examples. The feeding accuracy was evaluated by comparing backlash of least input increment, which was measured by counting the number of units necessary for shifting to the minus direction upon commanding to feed to the minus direction after commanding to feed to the plus direction. The test was carried out in an air-conditioned room at 24°C plus or minus 0.2°C. The machining centre was broken-in with the sample oil composition tested so as to lubricate the slideway surface sufficiently with the sample oil composition, and then the test was carried out 6 times. Then, the average of the results for each sample oil composition was obtained.

### Examples and Comparative Examples

The results of Examples 1 to 6 are shown in Table 1. The results of Comparative Examples 1 to 8, 11 and 12 are shown in Table 2.

Examples 1 to 6 relate to the lubricating oil composition of the present invention. Comparative Examples 1 to 6 relate to the lubricating oil compositions wherein no friction reducing agents were incorporated and/or wherein linear alkyl amines (c) of the present invention were deleted. Further, Comparative Examples 7 and 8 relate to the lubricating oil compositions wherein only specific linear alkyl amines were added. The results of the lubricating oil composition wherein branched alkyl amine was used instead of linear alkyl amine (c) were shown by Comparative Examples 11 and 12.

Comparisons of Example 1 with Comparative Example 3, Example 2 with Comparative Example 4, Example 3 with Comparative Example 5, and Examples 4, 5 and 6 with Comparative Example 6, indicate that lubricating oil compositions of the present invention (Examples 1 to 6) provide the machining centre with smaller backlash upon positioning and therefore, provides better positioning accuracy, compared with the lubricant oil compositions without linear alkyl amine (Comparative Examples 3 to 6).

Comparison of Comparative Examples 1 and 7 and comparison of Comparative Examples 2 and 8 show that lubricant oil compositions containing the linear alkyl amine (c) only do not improve positioning accuracy of the machining centre.

Comparison of Comparative Example 6 with Comparative Examples 11 and 12 indicates that the effect of the present invention cannot be obtained by using branched alkyl amines such as 2-ethylhexyl amine and tertiary C₁₆₋₂₂ amine instead of the linear alkyl amines (c).

**Table 1**

| | | Example | | | | | |
|---|---|---|---|---|---|---|---|
| | | 1 | 2 | 3 | 4 | 5 | 6 |
| Amine Salt of | 1 | - | - | - | 0.75 | 0.75 | 0.75 |
| Phosphoric Acid | 2 | - | 0.60 | - | - | - | - |
| Ester | 3 | - | - | 0.65 | - | - | - |
| Oleic Acid | | 0.25 | - | - | - | - | - |
| Sulfurised Lard | | - | - | 1.00 | - | - | - |
| Dioleyl Amine | | - | - | - | - | - | 0.01 |
| Lauryl Amine | | - | 0.01 | - | - | 0.01 | - |
| Oleyl Amine | | 0.01 | - | 0.01 | 0.01 | - | - |
| Backlash (number of | | 3 | 7 | 7 | 3 | 6 | 6 |
| input feed unit) | | | | | | | |

**Table 2**

| | | Comparative Example | | | | | | | | | |
|---|---|---|---|---|---|---|---|---|---|---|---|
| | | 1 | 2 | 3 | 4 | 5 | 6 | 7 | 8 | 11 | 12 |
| Amine Salt of | 1 | - | - | - | - | - | 0.75 | - | - | 0.75 | 0.75 |
| Phosphoric Acid | 2 | - | - | - | 0.60 | - | - | - | - | - | - |
| Ester | 3 | - | - | - | - | 0.65 | - | - | - | - | - |
| Oleic Acid | | - | - | 0.25 | - | - | - | - | - | - | - |
| Sulfurised Lard | | - | - | - | - | 1.00 | - | - | - | - | - |
| Tricresyl Phosphate | | - | 0.50 | - | - | - | - | - | 0.50 | - | - |
| 2-Ethylhexyl Amine | | - | - | - | - | - | - | - | - | - | 0.02 |
| tert-C₁₆₋₂₂ Alkyl Amine | | - | - | - | - | - | - | - | - | 0.01 | - |
| Oleyl Amine | | - | - | - | - | - | - | 0.01 | 0.01 | - | - |
| Backlash | | 12 | 12 | 6 | 11 | 11 | 8 | 12 | 12 | 9 | 8 |
| (number of input feed unit) | | | | | | | | | | | |

## Claims

1. A method of lubricating the slideway(s) of a machine tool or injection moulding machine comprising lubricating said slideway(s) with a lubricating oil composition comprising
(a) a base oil comprising one or more lubricating oils selected from mineral, vegetable and synthetic lubricating oils;
(b) one or more friction reducing agents selected from phosphoric acid ester alkyl ammonium salts of the formulae:
[(R¹O)ₙP(=O) (O⁻)₃₋ₙ] [R²ₘH₍₄₋ₘ₎N⁺]₃₋ₙ (1)
[(R¹O)ₙP(=O) (O⁻)₃₋ₙ] [R²ₘR³₍₃₋ₘ₎HN⁺]₃₋ₙ (2)
and fatty acids of the formulae: wherein
n is 1 or 2;
m is 1 to 3;
p is 1 to 10;
R¹ is a C₄₋₂₂ alkyl, alkenyl or alkynyl group, a C₆₋₂₄ alkylaryl group, an alkyl group to which 1 to 10 moles of polyoxyethylene is added, or an alkylaryl group to which 1 to 10 moles of polyoxyethylene is added;
R² is a C₄₋₂₆ alkyl, alkenyl or alkynyl group, a C₆₋₂₄ alkylaryl group or an aryl group;
R³ is a methyl or ethyl group;
R⁵ is a C₇₋₂₃ alkyl, alkenyl or alkynyl group or a sulphurised C₇₋₂₃ alkyl, alkenyl or alkynyl group;
R⁶ is a C₁₀₋₁₈ alkyl, alkenyl or alkynyl group; and
R⁷ is a C₈₋₁₈ alkyl, alkenyl or alkynyl group; and
(c) one or more linear alkyl amines selected from the amines represented by the formulae:
R⁸ₘ-N-H₍₃₋ₘ₎ (6)
wherein
m and R³ are as defined above; and
R⁸ is a linear C₈₋₂₂ alkyl, alkenyl or alkynyl group, provided that R⁸ has more carbon atoms than R² when R² is a linear alkyl, alkenyl or alkynyl group.

2. A method according to claim 1 wherein
R¹ is a C₄₋₂₀ alkyl group, a C₁₆₋₂₀ alkenyl group, a C₄₋₂₀ alkyl group to which 1 to 10 moles of polyoxyethylene is added, or a (C₁₋₁₀ alkyl)phenyl group to which 1 to 10 moles of polyoxyethylene is added;
R² is a C₄₋₁₆ alkyl group or a phenyl group;
R³ is a methyl group;
R⁵ is a C₈₋₂₀ alkyl group, a C₁₀₋₂₀ alkenyl group or a sulphurised C₁₆₋₁₈ alkenyl group;
R⁶ is a C₁₀₋₁₈ alkyl group or a C₁₆₋₂₀ alkenyl group;
R⁷ is a C₁₀₋₁₈ alkyl group; and
R⁸ is a linear C₈₋₂₀ alkyl group or C₁₆₋₂₀ alkenyl group.

3. A method according to claim 1 or 2 in which the one or more friction reducing agents (b) is/are present in an amount of 0.05 to 10% by weight based on the amount of base oil (a) in the composition.

4. A method according to any one of claims 1 to 3 in which the one or more linear alkyl amines (c) is/are present in the amount of 0.1 to 20% by weight based on the amount of friction reducing agent (s) (b) in the composition.

5. A method according to claim 4 in which the one or more linear alkyl amines (c) is/are present in the amount of 1 to 10% by weight based on the amount of friction reducing agent(s) (b) in the composition.

6. Use of a lubricating oil composition as defined in any one of claims 1 to 5 for lubricating the slideway(s) of a machine tool or injection moulding machine.

## Patentansprüche

1. Verfahren zur Schmierung der Gleitbahn (Gleitbahnen) eines Maschinenwerkzeuges oder einer Spritzgußmaschine, umfassend das Schmieren der Gleitbahn (Gleitbahnen) mit einer Schmierölzusammensetzung, umfassend
(a) ein Grundöl, umfassend eines oder mehrere Schmieröle, welche unter mineralischen, pflanzlichen und synthetischen Schmierölen ausgewählt sind;
(b) eines oder mehrere die Reibung verringernde Mittel, ausgewählt unter Phosphorsäureesteralkylammoniumsalzen der Formeln:
[(R¹O)ₙP(=O) (O⁻)₃₋ₙ] [R²ₘH₍₄₋ₘ₎N⁺]₃₋ₙ (1)
[(R¹O)ₙP(=O) (O⁻)₃₋ₙ] [R²ₘR³₍₃₋ₘ₎HN⁺]₃₋ₙ (2)
und Fettsäuren der Formeln: worin
n 1 oder 2 beträgt;
m 1 bis 3 beträgt;
p 1 bis 10 beträgt;
R¹ eine C₄₋₂₂-Alkyl-, -Alkenyl- oder -Alkinylgruppe, eine C₆₋₂₄-Alkylarylgruppe, eine Alkylgruppe, an welche 1 bis 10 Mol Polyoxyethylen addiert sind, oder eine Alkylarylgruppe, an welche 1 bis 10 Mol Polyoxyethylen addiert sind, darstellt;
R² eine C₄₋₂₆-Alkyl-, -Alkenyl- oder -Alkinylgruppe, eine C₆₋₂₄-Alkylarylgruppe oder eine Arylgruppe bedeutet;
R³ für eine Methyl- oder Ethylgruppe steht;
R⁵ eine C₇₋₂₃-Alkyl-, -Alkenyl- oder -Alkinylgruppe oder eine sulfurierte C₇₋₂₃-Alkyl-, -Alkenyl- oder -Alkinylgruppe bedeutet;
R⁶ eine C₁₀₋₁₈-Alkyl-, -Alkenyl- oder -Alkinylgruppe darstellt; und
R⁷ eine C₈₋₁₈-Alkyl-, -Alkenyl- oder -Alkinylgruppe bedeutet; und
(c) ein oder mehrere lineare Alkylamine, ausgewählt unter den Aminen, welche durch die Formeln:
R⁸ₘ-N-H₍₃₋ₘ₎ (6)
dargestellt werden, worin
m und R³ wie vorstehend definiert sind; und
R⁸ eine lineare C₈₋₂₂-Alkyl-, -Alkenyl- oder -Alkinylgruppe darstellt, mit der Maßgabe, daß R⁸ mehr Kohlenstoffatome als R² besitzt, wenn es sich bei R² um eine lineare Alkyl-, Alkenyl- oder Alkinylgruppe handelt.

2. Verfahren nach Anspruch 1, worin
R¹ eine C₄₋₂₀-Alkylgruppe, eine C₁₆₋₂₀-Alkenylgruppe, eine C₄₋₂₀-Alkylgruppe, an welche 1 bis 10 Mol Polyoxyethylen addiert sind, oder eine (C₁₋₁₀-Alkyl)phenylgruppe darstellt, an welche 1 bis 10 Mol Polyoxyethylen addiert sind;
R² eine C₄₋₁₆-Alkylgruppe oder eine Phenylgruppe bedeutet;
R³ eine Methylgruppe ist;
R⁵ eine C₈₋₂₀-Alkylgruppe, eine C₁₀₋₂₀-Alkenylgruppe oder eine sulfurierte C₁₆₋₁₈-Alkenylgruppe darstellt;
R⁶ eine C₁₀₋₁₈-Alkylgruppe oder eine C₁₆₋₂₀-Alkenylgruppe bedeutet;
R⁷ eine C₁₀₋₁₈-Alkylgruppe darstellt; und
R⁸ eine lineare C₈₋₂₀-Alkylgruppe oder eine C₁₆₋₂₀-Alkenylgruppe bedeutet.

3. Verfahren nach Anspruch 1 oder 2, worin das eine oder die mehreren die Reibung verringernden Mittel (b) in einer Menge von 0,05 bis 10 Gew.-%, bezogen auf die Menge an Grundöl (a) in der Zusammensetzung, vorhanden ist/sind.

4. Verfahren nach einem der Ansprüche 1 bis 3, worin das eine oder die mehreren linearen Alkylamine (c) in einer Menge von 0,1 bis 20 Gew.-%, bezogen auf die Menge an die Reibung verringerndem Mittel (die Reibung verringernden Mitteln) (b) in der Zusammensetzung, vorhanden ist/sind.

5. Verfahren nach Anspruch 4, worin das eine oder die mehreren linearen Alkylamin(e) (c) in einer Menge von 1 bis 10 Gew.-%, bezogen auf die Menge an die Reibung verringerndem Mittel (die Reibung verringernden Mitteln) (b) in der Zusammensetzung, vorhanden ist/sind.

6. Verwendung einer Schmierölzusammensetzung, wie sie in einem der Ansprüche 1 bis 5 definiert ist, zur Schmierung der Gleitbahn (Gleitbahnen) eines Maschinenwerkzeugs oder einer Spritzgußmaschine.

## Revendications

1. Procédé de lubrification de la ou des glissières d'une machine-outil ou d'une machine de moulage par injection comprenant la lubrification de ladite ou desdites glissières avec une composition d'huile lubrifiante comprenant :
(a) une huile de base comprenant une ou plusieurs huiles lubrifiantes choisies parmi les huiles lubrifiantes minérales, végétales et synthétiques;
(b) un ou plusieurs agents de réduction de friction choisis parmi les sels d'alkyl ammonium d'esters d'acide phosphorique des formules :
[(R¹O)ₙP(=O)(O⁻)₃₋ₙ][R²ₘH₍₄₋ₘ₎N⁺]₃₋ₙ (1)
[(R¹O)ₙP(=O)(O⁻)₃₋ₙ][R²ₘR³₍₃₋ₘ₎HN⁺]₃₋ₙ (2)
et les acides gras des formules : dans lesquelles :
n est égal à 1 ou 2;
m vaut de 1 à 3;
p vaut de 1 à 10;
R¹ est un groupe alkyle, alcényle ou alcynyle en C₄₋₂₂, un groupe alkylaryle en C₆₋₂₄, un groupe alkyle auquel 1 à 10 moles de polyoxyéthylène sont ajoutées, ou un groupe alkylaryle auquel 1 à 10 moles de polyoxyéthylène sont ajoutées;
R² est un groupe alkyle, alcényle ou alcynyle en C₄₋₂₆, un groupe alkylaryle en C₆₋₂₄ ou un groupe aryle;
R³ est un groupe méthyle ou éthyle;
R⁵ est un groupe alkyle, alcényle ou alcynyle en C₇₋₂₃ ou un groupe alkyle, alcényle ou alcynyle en C₇₋₂₃ sulfurisé;
R⁶ est un groupe alkyle, alcényle ou alcynyle en C₁₀₋₁₈; et
R⁷ est un groupe alkyle, alcényle ou alcynyle en C₈₋₁₈; et
(c) une ou plusieurs alkyl amines linéaires choisies parmi les amines représentées par les formules :
R⁸ₘ-N-H₍₃₋ₘ₎ (6)
dans lesquelles :
m et R³ sont tels que définis précédemment; et
R⁸ est un groupe alkyle, alcényle ou alcynyle en C₈₋₂₂ linéaire, pour autant que R⁸ comporte plus d'atomes de carbone que R² lorsque R² est un groupe alkyle, alcényle ou alcynyle linéaire.

2. Procédé suivant la revendication 1, dans lequel :
R¹ est un groupe alkyle en C₄₋₂₀, un groupe alcényle en C₁₆₋₂₀, un groupe alkyle en C₄₋₂₀ auquel 1 à 10 moles de polyoxyéthylène sont ajoutées, ou un groupe (alkyl en C₁₋₁₀)phényle auquel 1 à 10 moles de polyoxyéthylène sont ajoutées;
R² est un groupe alkyle en C₄₋₁₆ ou un groupe phényle;
R³ est un groupe méthyle;
R⁵ est un groupe alkyle en C₈₋₂₀, un groupe alcényle en C₁₀₋₂₀ ou un groupe alcényle en C₁₆₋₁₈ sulfurisé;
R⁶ est un groupe alkyle en C₁₀₋₁₈ ou un groupe alcényle en C₁₆₋₂₀;
R⁷ est un groupe alkyle en C₁₀₋₁₈; et
R⁸ est un groupe alkyle en C₈₋₂₀ ou un groupe alcényle en C₁₆₋₂₀ linéaire.

3. Procédé suivant l'une ou l'autre des revendications 1 et 2, dans lequel le ou les plusieurs agents de réduction de friction (b) est (sont) présent en une quantité de 0,05 à 10 % en poids par rapport à la quantité d'huile de base (a) dans la composition.

4. Procédé suivant l'une quelconque des revendications 1 à 3, dans lequel la ou les plusieurs alkyl amines linéaires (c) est (sont) présente en la quantité de 0,1 à 20 % en poids par rapport à la quantité d'agent(s) de réduction de friction (b) dans la composition.

5. Procédé suivant la revendication 4, dans lequel la ou les plusieurs alkyl amines linéaires (c) est (sont) présente en la quantité de 1 à 10 % en poids par rapport à la quantité d'agent(s) de réduction de friction (b) dans la composition.

6. Utilisation d'une composition d'huile lubrifiante suivant l'une quelconque des revendications 1 à 5 pour lubrifier la ou les glissières d'une machine-outil ou d'une machine de moulage par injection.
